

## 1

2,904,177

## FLOTATION OF SILICATES FROM TITANIFEROUS IRON ORES

Eugene J. Michal, Metuchen, N.J., assignor to National Lead Company, New York, N.Y., a corporation of New Jersey

No Drawing. Application May 29, 1957  
Serial No. 662,322

4 Claims. (Cl. 209—166)

This invention relates in general to the treatment of a titaniferous iron material. More specifically, it relates to a flotation method for the removal of silicates from a titaniferous iron ore.

Many methods have been used in the past for separating the silicates and other constituents from the titanium bearing materials in a titaniferous iron ore. Among the most useful methods are flotation processes in which the silicates are separated from the titanium values by adding anionic type promotors to the ore and floating off the titanium values from the silicates. This operation is usually carried out under neutral or slightly alkaline conditions. The most useful anionic type promotors are oleic acid, fish oil, fatty acids, resin or naphthenic acids and the like.

Although these methods have met with some success when processing various types of ore, however, these processes are not too successful with ilmenite ores since the ilmenite fraction often constitutes the bulk of the ore and has to be floated away from the silicate values. Since the silicate portion of an ilmenite ore is, in many instances, less than the ilmenite fraction, it would be desirable to employ a process where the silicate portion is removed by flotation from the ilmenite values.

An object of the instant invention, therefore, is to provide a simple and economical method for separation of silicates from ilmenite ore. A further object is to provide a straightforward flotation method for the separation of silicates from the ilmenite values. These and other objects will become apparent from the following more complete description of the instant invention.

Broadly, this invention contemplates a process for separating silicates from the titanium values in an ilmenite ore which comprises grinding the ore to —60 mesh size, preparing an aqueous pulp with said ground ore, acidifying said pulp to a pH between 3.0 and 6.0 by adding hydrofluoric acid, adding starch to said pulp to depress the titanium values adding to said pulp a cationic amine flotation agent and subjecting the treated pulp to a froth flotation whereby said silicates are removed by flotation from the residual titanium values.

The silicate portion of the ore which is to be removed by the flotation operation from the ilmenite portion usually consists of a number of mineral constituents. The most common of these silicates present in the ore are garnet, feldspars, hornblende and augite.

Ilmenite ores usually contain various amounts of these silicate constituents which cannot be removed by mechanical means such as grinding, magnetic separation, gravity concentration, and the like and, therefore a flotation process is useful. The flotation process of the instant invention is particularly desirable since the silicate, usually the smaller portion, is floated away from the ilmenite fraction.

## 2

In carrying out the process of the instant invention, the ilmenite ore containing the silicates to be removed was ground until the ore passed through a 60 mesh size screen. A pulp of the ground ore was prepared in water, 5 the pulp density was 20% to 50% solids. If desired, the ground ore was deslimed before forming the pulp slurry in order to obtain a more complete flotation separation.

The pulp was acidified to a pH of 3.0 to 6.0 with 10 either hydrofluoric acid or a mixture of hydrofluoric acid and sulfuric acid. During the flotation run further acid was added, if necessary, to maintain the acidity within the specified pH range. The presence of hydrofluoric acid is necessary to remove the feldspars and other silicates, however, for economy it is desirable to employ a mixture of hydrofluoric and sulfuric acids.

Starch was added to the acidified pulp to depress the ilmenite. Several types of starches, such as arrowroot, wheat, tapioca, and corn, were satisfactory but potato 20 starch seemed to be particularly effective. The starch was added for convenience as a one percent solution in amounts ranging from 0.5 to 20.0 pounds of starch per ton of ore.

After the ilmenite was depressed, a cationic amine 25 flotation agent was added as a collector of the silicates in the ore. Illustrative examples of the cationic amine flotation agents which are particularly effective are higher aliphatic amines, such as lauryl amine, hexadecyl amine, dodecyl amine, short chain amines such as triethanol amine; amine salts which may be used include lauryl amine hydrochloride, hexadecyl amine hydrochloride, and dodecyl amine hydrochloride; quaternary ammonium salts of the higher aliphatic series may be used such as cetyl trimethyl ammonium bromide, lauryl triethyl ammonium chloride and octadecyl trimethyl ammonium chloride. Commercial grade fatty amine acetates may be used such as Armac CD and Armac TD made by Armour and Company, or primary and secondary fatty amines such as Armeen CD and Armeen TD made 35 by Armour and Company or a primary amine derivative of dehydroabietylamine such as rosin amine D acetate made by Hercules Powder Company. The fatty amine acetates, Armac CD and Armac TD are alkylammonium acetates having the general formula:



The fatty amines, Armeen CD and Armeen TD are primary and secondary fatty amines having the following 40 formulae:



The molecular weights, melting points and composition 45 of the amine content of these cationic agents are as follows:

|    | Properties                 | Armac CD | Armac TD | Armeen CD | Armeen TD |
|----|----------------------------|----------|----------|-----------|-----------|
| 60 | Mean molecular weight..... | 226      | 331      | 200       | 263       |
|    | Melting point, °C.....     | 55       | 65       | 21        | 41        |
|    | Percent octyl.....         | 8        | —        | 8         | —         |
|    | Percent decyl.....         | 9        | —        | 9         | —         |
|    | Percent dodecyl.....       | 47       | —        | 47        | —         |
|    | Percent tetradecyl.....    | 18       | —        | 18        | —         |
|    | Percent hexadecyl.....     | 8        | 30       | 8         | 30        |
| 65 | Percent octadecyl.....     | 5        | 25       | 5         | 25        |
|    | Percent octadecenyl.....   | 5        | 45       | 5         | 45        |

The rosin amine D acetate identified as RADA made by Hercules Powder Company is the reaction product

## 3

of acetic acid and dehydroabietylamine having the following structural formula:



The amount of collector added should be from 0.2 to 1.0 pound per ton of ore treated. These cationic flotation agents usually act as their own frother, however, pine oil and other frothers may be added in addition if desired.

After sufficient aeration a relatively clean separation between the silicate portion and the ilmenite portion was obtained.

If it is desired to further separate the two fractions from one another, the above operation may be repeated and a more complete separation will be obtained.

In order to further illustrate the process of the instant invention, the following examples are presented.

## Example I

An ilmenite concentrate had the following mineral composition:

|                            | Percent |
|----------------------------|---------|
| Ilmenite                   | 87      |
| Garnet                     | 4       |
| Feldspar                   | 2       |
| Hornblende                 | 3       |
| Augite                     | 3       |
| Sulfides                   | 0.5     |
| Miscellaneous <sup>1</sup> | 0.5     |

<sup>1</sup> Includes mica, spinel, and unidentified minerals.

Twenty-two hundred grams of this ilmenite concentrate was disc pulverized to minus 60 mesh, and added to 2,000 ml. of water in a laboratory flotation machine.

The slurry was made basic with sodium carbonate and the sulfide minerals were floated with a xanthate reagent according to established practice for bulk flotation of sulfide minerals. The tailings or residue in the flotation machine were then deslimed by stopping the agitation, and one to two minutes later the water was decanted with the finely suspended material. The tailings were twice repulped with 2,000 ml. of water and the slimes were decanted.

After the desliming treatment, the ore residue in the flotation machine was made up to about 50% solids by addition of tap water, and the following reagents were used in the flotation procedure:

3.6 lbs. hydrofluoric acid per ton of ilmenite concentrate  
0.6 lb. sulfuric acid per ton of ilmenite concentrate  
1.45 lbs. potato starch (1% water solution) per ton of ilmenite concentrate

0.70 lb. RADA (Rosin Amine D Acetate—Hercules Powder Co.) per ton of ilmenite concentrate.

To the ore slurry in the flotation machine were added 3.6 lbs. per ton of hydrofluoric acid to bring the pH down to 3.5. The slurry was conditioned (agitated) for three minutes after which 1.3 lbs. per ton of starch were added, and conditioned for three minutes. Next, 0.28 pound per ton of RADA was added and conditioned for five minutes. Air was admitted, and a froth carrying the silicate minerals was removed. At this stage the pH of the pulp was about 4.0. Three further steps of reagent addition and froth flotation were carried out. The first, involved the addition of 0.14 pound per ton of RADA only. The second, addition of 0.30 pound per ton of  $H_2SO_4$ , 0.10 pound per ton of potato starch,

and 0.14 pound per ton of RADA. The third step was the addition of 0.30 pound per ton of  $H_2SO_4$ , 0.05 pound per ton of starch, and 0.14 pound per ton of RADA.

At the end of the test the pH of the slurry was 3.5.

5 The products of the test were as follows:

|    | Product             | Weight (grams) | Percent $TiO_2$ | $TiO_2$ distribution |
|----|---------------------|----------------|-----------------|----------------------|
| 10 | Sulfide concentrate | 10             | 21.4            | 0.22                 |
|    | Slimes              | 153            | 40.6            | 6.35                 |
|    | Flotation froth     | 211            | 3.9             | 0.84                 |
|    | Flotation tails     | 1,822          | 49.6            | 92.60                |
|    |                     | 2,196          | 44.5            | 100.01               |

Only 3.4% silicates remained in the flotation tails which represented a 79% removal by the flotation process.

## Example II

20 Another ilmenite ore had the following mineral composition:

|                            | Percent |
|----------------------------|---------|
| Ilmenite                   | 61.1    |
| Feldspar                   | 13.7    |
| 25 Hornblende              | 13.7    |
| Garnet                     | 5.5     |
| Augite                     | 4.6     |
| Miscellaneous <sup>1</sup> | 1.4     |

<sup>1</sup> Includes mica, spinel, sulfides, and unidentified minerals.

30 Eleven hundred grams of this ore were wet ball-milled in a steel mill at about 50 percent solids pulp density to about 80 percent minus 100 mesh. The milled slurry was added to a laboratory flotation machine and water was added to make a pulp density of about 25 percent solids.

To the agitated pulp were added the following reagents in the order listed:

- 35 3.5 pounds hydrofluoric acid per ton of ilmenite ore  
40 2.0 pounds potato starch (1% water solution) per ton of ilmenite ore  
0.76 pound of RADA (Rosin Amine D acetate Hercules Powder Co.) per ton of ilmenite ore  
0.06 pound of pine oil per ton of ilmenite ore

45 Three minutes conditioning time was allowed after each reagent addition. Air was admitted to the flotation machine and the mineral froth was removed.

The products of the test were as follows:

|    | Product           | Weight (grams) | Percent $TiO_2$ | $TiO_2$ distribution |
|----|-------------------|----------------|-----------------|----------------------|
| 55 | Flotation froth   | 413            | 10.6            | 13.4                 |
|    | Flotation tailing | 662            | 42.8            | 86.6                 |
|    | Calculated head   | 1,075          | 30.4            | 100.0                |

50 This represented about a 75% removal of the silicate values by the flotation process.

## Example III

Another type of an ilmenite ore had the following mineral composition:

|                            | Percent |
|----------------------------|---------|
| 65 Magnetite               | 57      |
| Ilmenite                   | 25      |
| Feldspar                   | 6       |
| 70 Hornblende              | 6       |
| Garnet                     | 3       |
| Augite                     | 2       |
| Miscellaneous <sup>1</sup> | 1       |

<sup>1</sup> Includes mica, spinel, sulfides, and unidentified minerals.

75 Twelve hundred grams of this ore were disc pulverized

to a size of about -60 mesh, and added to 2,500 ml. of water in a laboratory flotation machine.

The slurry was agitated and the following reagents were added:

7.0 pounds hydrofluoric acid per ton of ilmenite ore  
3.3 pounds potato starch per ton of ilmenite ore  
0.80 pound of RADA (Rosin Amine D Acetate—Hercules Powder Company) per ton of ilmenite ore

The 0.80 pound of RADA was added in three separate increments with a conditioning period of three minutes after each addition.

Air was admitted to the flotation machine after each of the three RADA reagent additions and the froth was removed. The products of the test were as follows:

| Product           | Weight (grams) | Percent $TiO_2$ | Percent $Fe(OH)_3$ | $TiO_2$ distribution |
|-------------------|----------------|-----------------|--------------------|----------------------|
| Flotation froth   | 310            | 10.6            | 18.4               | 14.7                 |
| Flotation tailing | 845            | 22.6            | 49.0               | 85.3                 |
| Calculated head   | 1,155          | 19.4            | 40.8               | 100.0                |

This represented about a 71% silicate removal by the flotation process.

#### Example IV

One thousand grams of the ilmenite concentrate described in Example I was disc pulverized to about 60 mesh and added to 2,500 ml. of water in a laboratory flotation machine. The mixture was agitated and then agitation stopped and the slurry allowed to settle for 1 to 2 minutes, after which time the slimes or fines remaining in suspension were decanted. This procedure was repeated twice, and after the third decantation sufficient water was again added to make an agitated pulp density of about 30% solids.

The following reagents were added to the agitated slurry in the order listed:

1.5 pounds of potato starch (1% water solution) per ton of concentrate  
2.4 pounds of hydrofluoric acid per ton of concentrate  
2.0 pounds of Armeen TD (Armour & Co.) per ton of concentrate  
0.062 pound of pine oil per ton of concentrate

One minute conditioning time was allowed between the additions of the several reagents. Air was admitted to the flotation machine and the froth was removed.

The products of the test were as follows:

| Product         | Weight (grams) | Percent $TiO_2$ | $TiO_2$ distribution |
|-----------------|----------------|-----------------|----------------------|
| Slimes          | 210            | 41.7            | 19.7                 |
| Flotation froth | 47             | 6.6             | 0.7                  |
| Flotation tails | 732            | 48.4            | 79.6                 |
| Calculated head | 989            | 45.0            | 100.0                |

The silicate removal by flotation was about 50%.

#### Example V

One thousand grams of the ilmenite concentrate described in Example I was disc pulverized to about 60 mesh and added to 2,000 ml. of water in a laboratory flotation machine.

Agitation was begun and the following reagents were added to the slurry in the order listed:

1.52 pounds potato starch (1% water solution) per ton of concentrate  
2.4 pounds hydrofluoric acid per ton of concentrate  
0.5 pound Armac CD (Armour and Co.) per ton of concentrate  
0.062 pound pine oil per ton of concentrate

The 0.5 pound of Armac CD was added in three increments with conditioning after each addition.

One minute conditioning time was allowed between additions of the several reagents. Air was admitted to the flotation machine and the froth was removed.

The products of the test were as follows:

| Product           | Weight (grams) | Percent $TiO_2$ | $TiO_2$ distribution |
|-------------------|----------------|-----------------|----------------------|
| Flotation froth   | 180            | 23.2            | 9.5                  |
| Flotation tailing | 800            | 49.6            | 90.5                 |
| Calculated head   | 980            | 44.7            | 100.0                |

15 The silicate removal by flotation was about 79%.

#### Example VI

An ilmenite concentrate had the following mineral composition:

|                            | Percent |
|----------------------------|---------|
| Ilmenite                   | 83      |
| Garnet                     | 5       |
| Feldspar                   | 3       |
| Hornblende & Augite        | 8       |
| Miscellaneous <sup>1</sup> | 1       |

<sup>1</sup> Includes mica, spinel, sulfides and unidentified minerals.

Twenty-two hundred grams of this ilmenite concentrate were wet ground in a steel ball mill at 50% solids with 0.227 pound of Aerosol OS (American Cyanamid Company) per ton of concentrate. The milled product was transferred to a laboratory flotation machine and the sulfide minerals floated out in a basic circuit with a xanthate reagent according to established practices for bulk flotation of sulfide minerals.

To the agitated slurry which remained in the flotation cell were added the following reagents in a flotation procedure:

|                                                                                                                  |                                                      |
|------------------------------------------------------------------------------------------------------------------|------------------------------------------------------|
| 40                                                                                                               | 4.36 pounds hydrofluoric acid per ton of concentrate |
| 2.55 pounds potato starch (1% water solution) per ton of concentrate                                             |                                                      |
| 0.655 pound of 50% water solution of RADA (Rosin Amine D Acetate—Hercules Powder Company) per ton of concentrate |                                                      |
| 0.025 pound of pine oil per ton of concentrate                                                                   |                                                      |

The reagents were added in three steps, in the following order: 3.27 pounds of HF per ton of ore, followed by one minute conditioning to give a pH of about 4.0 in the slurry; 1.82 pounds of starch per ton of ore, followed by two minutes conditioning; three additions of 0.145 pound of RADA per ton of ore, with 30 seconds conditioning after each addition; and 0.73 pound of starch per ton of ore. Air was admitted, and a flotation froth removed. The second stage of reagent addition was begun immediately, and 1.09 pounds of HF per ton of ore, 0.145 pound of RADA per ton of ore, and 0.025 pound of pine oil per ton of ore were added. Air was admitted and a second flotation froth removed.

The third stage of reagent addition was immediately carried out and consisted of the addition of 0.072 pound of RADA per ton of ore. A third froth was removed by admitting air to the machine, and this completed the flotation.

65 The products of the test were as follows:

| Product         | Weight (grams) | Percent $TiO_2$ | $TiO_2$ distribution |
|-----------------|----------------|-----------------|----------------------|
| Sulfide float   | 110            | 35.7            | 4.2                  |
| Silicate float  | 345            | 16.75           | 6.2                  |
| Tails           | 1,705          | 49.0            | 89.6                 |
| Calculated head | 2,160          | 43.2            | 100.0                |

A 75% silicate removal was obtained in the silicate flotation step.

*Example VII*

Six hundred grams of the ilmenite concentrate described in Example I were disc pulverized to -60 mesh and added to 2,000 ml. of water in a laboratory flotation machine.

Agitation was begun and the slurry was treated with the following flotation reagents:

14.0 pounds wheat starch per ton of concentrate  
7.2 pounds hydrofluoric acid per ton of concentrate  
0.56 pound of RADA (Rosin Amine D Acetate—Hercules Powder Co.) per ton of concentrate.  
0.12 pound of pine oil per ton of concentrate

The reagents were added in the order listed above, with 1-3 minutes conditioning time between reagent additions. Air was admitted to the flotation machine and a froth removed.

The products of the test were as follows:

| Product                | Weight (grams) | Percent $TiO_2$ | $TiO_2$ distribution |
|------------------------|----------------|-----------------|----------------------|
| Flotation froth.....   | 218            | 37.45           | 32.3                 |
| Flotation tailing..... | 347            | 49.35           | 67.7                 |
| Calculated head.....   | 565            | 44.70           | 100.0                |

This represented about an 81% removal of the silicate minerals.

*Example VIII*

Six hundred grams of the ilmenite concentrate described in Example I were disc pulverized to about 60 mesh and added to 2,000 ml. of water in a laboratory flotation machine.

Agitation was begun and the following reagents were added to the slurry in the order listed:

18.0 pounds of arrowroot starch per ton of concentrate  
7.2 pounds hydrofluoric acid per ton of concentrate  
2.0 pounds Armeen TD (Armour and Co.) per ton of concentrate  
0.88 pound RADA (Rosin Amine D Acetate—Hercules Powder Company) per ton of concentrate

The RADA was added in three separate increments. One to three minutes conditioning time was allowed between the additions of the several agents. Air was admitted to the flotation machine and a froth was removed subsequent to each of the three increments of RADA addition.

The products of the test were as follows:

| Product                | Weight (grams) | Percent $TiO_2$ | $TiO_2$ distribution |
|------------------------|----------------|-----------------|----------------------|
| Flotation froth.....   | 186            | 35.25           | 25.9                 |
| Flotation tailing..... | 378            | 49.7            | 74.1                 |
| Calculated head.....   | 564            | 44.9            | 100.0                |

About 83% of the silicates were removed by flotation. From the above description and by the examples presented, it has clearly been shown that efficient silicate removal from ilmenite ore has been obtained by utilizing the process of the instant invention. The flotation process of the instant invention is particularly effective in removing the silicate values from an ilmenite ore because the lesser quantities of silicate minerals are floated away from the ilmenite values. With ilmenite ores and concentrates, the silicate content is often much less than the ilmenite content and, therefore, the process of the instant invention is more effective than the prior art methods which remove by flotation the ilmenite portion from the silicate portion. The process of the instant invention is a simple and economical operation which results in efficient removal of the silicate fractions.

While this invention has been described and illustrated by the examples shown, it is not intended to be strictly limited thereto, and other modifications and variations may be employed within the scope of the following claims.

I claim:

1. A method for separating silicates from the titanium values in a titaniferous iron ore which comprises grinding the ore to -60 mesh size, pulping the ground ore in aqueous media, acidifying the pulp to a pH between about 3.0 and 6.0 by adding thereto an acid solution containing an ionizable fluoride ion, adding starch to said acidified pulp to depress the titanium values, adding to said pulp a cationic amine flotation agent in amount from 0.2 to 1.0 pound per ton of ore and subjecting the treated pulp to a froth flotation whereby said silicates are removed by flotation from the residual titanium values.
2. Method according to claim 1 in which the titaniferous iron ore is ilmenite ore.
3. Method according to claim 1 in which the pulp is acidified with a combination of hydrofluoric acid and sulfuric acid.
4. Method according to claim 1 in which the amount of starch employed is from 0.5 to 20.0 pounds per ton of ore.

References Cited in the file of this patent

UNITED STATES PATENTS

|           |                     |               |
|-----------|---------------------|---------------|
| 2,297,689 | O'Meara .....       | Oct. 6, 1942  |
| 2,410,021 | De Vaney .....      | Oct. 29, 1946 |
| 2,466,995 | McMurray .....      | Apr. 12, 1949 |
| 2,483,890 | De Vaney .....      | Oct. 4, 1949  |
| 2,666,588 | Schack et al. ..... | Jan. 19, 1954 |
| 2,792,940 | Baarson .....       | May 21, 1957  |

OTHER REFERENCES

Chang: "Substituted Starches in Amine Flotation of Iron Ore," Mining Engineering, September 1954, pages 922-924.